

## UNITED STATES PATENT OFFICE

STEPHAN JOST, OF BASEL, SWITZERLAND, ASSIGNOR TO THE FIRM, FARBEREI- & OPPRETUR GESELLSCHAFT (VORMALS A. BLAVEL & FRITZ LINDEMAYER), OF BASEL, SWITZERLAND

## TREATMENT OF SILK

No Drawing. Application filed January 16, 1925, Serial No. 2,938, and in Germany November 8, 1924.

A problem of great interest in the silk industry is the durability of weighted silk. The protective treatments hitherto known have been based on the action of reducing substances, such as thiosulphates, formaldehyde bisulphite, hydroxylamine, hydroquinone or thio-urea. These treatments require operation in acid solutions. On the other hand it has been proposed to protect weighted silk by a subsequent treatment with an ammonia-formaldehyde preparation or rhodan compounds, but it has been observed in this case that these compounds produce undesirable color modifications or spots. Further it is well known that after acid metal salt solutions an alkaline treatment is used with alkali phosphate or carbonate which belongs to the weighting proper process and serves only to fix the mordant salt and does not concern the final reaction after dyeing. By the present invention, however, a moderately long treatment of the silk after complete weighting and in the course of subsequent dyeing, printing and finishing operations in an additional alkaline bath free from formaldehyde and rhodan, such as a solution of ammonia, of a phosphate (trisodium phosphate), of a borate, of an organic base and so on, produces very good protective effects in respect of rotting under the influence of both light and temperature without affecting the color or other properties of the silk. The fundamental novelty of the invention is derived from the observation that weighted silk fibre when in a neutral or feebly alkaline condition exhibits far greater resistance to the chemical processes which occur during storage than if there is present even a trace of acid. Researches, made by the inventor, show that best results are obtained when the concentration of H-ions, determined in an aqueous extract of the fiber, ranges between min. pH 7.0 and max. pH 10. (Temperature of determination 20° C.).

The effect of the invention is surprising. For example, the tensile strength of the weft of a normal dyed weft-silk, tied with the sarsenet ribbon, after 4 months storage in a tropical climate in a place protected

from direct solar radiation, diminished from 20.7 kilos to 10.4 kilos, whereas the silk which had been treated by this invention diminished in tensile strength only to an insignificant amount, namely from 19.6 kilos to 19.1. These figures show the technical advance made by the invention without further demonstration. There is no effect on the lustre of the fibre and the effect on the feel of the material is such that it cannot be regarded as technically disadvantageous but rather as an improvement for certain purposes.

The invention can be applied to silk in hanks or piece goods, or in mixed fabrics, after the weighting operation is finished, during or after the dyeing, printing and finishing. The essential being that the additional alkaline bath is capable of rendering the fiber free from acid substances by producing min. pH 7.0 to max. pH 10, determined in an aqueous extract of the fiber at 20° C.

The following examples illustrate the invention:—

## Example 1

The weighted silk after dyeing is washed and treated on a boiled-off liquor bath, that is a soap solution containing sericin, at 40° C. for half an hour with about 5 grams of soap per litre and only so much ammonia as is necessary to eliminate all acid reaction in the fibre; any necessary washing follows. In the case of dark dyeings the treatment may be carried out even in the cold.

## Example 2

The silk receives after the operation of weighting it with water glass, as usual, two soap baths at 50° C., there being added to the second bath in dyeing operation 5 grams of trisodium-phosphate per litre of the liquor, and in some cases, particularly for light tints, the necessary dyestuffs for the dyeing, whilst for darker shades the dyestuffs may be added in a following bath. A subsequent treatment with acid is not permissible.

*Example 3*

The weighted and dyed silk in hank or web is treated in the usual manner with a dressing solution consisting of an alkaline solution of tragacanth in combination with  $\beta$ -naphthylamine as a feeble base; only a feebly alkaline reaction of the fibre is produced.

5 **What I claim is:**

10 1. A method for increasing the permanence and stability of completely weighted and dyed silk fibre consisting in treating the fibre with a basic bath free from formaldehyde compounds, after the weighting, to neutralize any remaining acidity of the fibre.

15 2. A method for increasing the permanence and stability of completely weighted and dyed silk fibre consisting in treating the same with a bath which contains an inorganic base and which is free from formaldehyde compounds, after the weighting, to neutralize any remaining acidity of the fibre.

20 25 3. A method for increasing the permanence and stability of completely weighted and dyed silk fibre consisting in treating the same with a bath which contains ammonia, but is free from formaldehyde compounds, after the weighting.

30 35 4. A method for increasing the permanence and stability of completely weighted and dyed silk fibre consisting in treating the same with a bath which contains inorganic alkaline salts, but is free from formaldehyde compounds, after the weighting.

35 40 5. A method for increasing the permanence and stability of completely weighted and dyed silk fibre consisting in treating the same with a bath which contains disodium phosphate but is free from formaldehyde compounds, after the weighting.

45 In witness whereof I have hereunto signed my name this 3rd day of January 1925.

STEPHAN JOST.

*Example 3*

The weighted and dyed silk in hank or web is treated in the usual manner with a dressing solution consisting of an alkaline solution of tragacanth in combination with  $\beta$ -naphthylamine as a feeble base; only a feebly alkaline reaction of the fibre is produced.

10 What I claim is:

1. A method for increasing the permanence and stability of completely weighted and dyed silk fibre consisting in treating the fibre with a basic bath free from formaldehyde compounds, after the weighting, to neutralize any remaining acidity of the fibre.

2. A method for increasing the permanence and stability of completely weighted and dyed silk fibre consisting in treating the same with a bath which contains an inorganic base and which is free from formaldehyde compounds, after the weighting, to neutralize any remaining acidity of the fibre.

3. A method for increasing the permanence and stability of completely weighted and dyed silk fibre consisting in treating the same with a bath which contains ammonia, but is free from formaldehyde compounds, after the weighting.

4. A method for increasing the permanence and stability of completely weighted and dyed silk fibre consisting in treating the same with a bath which contains inorganic alkaline salts, but is free from formaldehyde compounds, after the weighting.

5. A method for increasing the permanence and stability of completely weighted and dyed silk fibre consisting in treating the same with a bath which contains disodium phosphate but is free from formaldehyde compounds, after the weighting.

In witness whereof I have hereunto signed my name this 3rd day of January 1925.

STEPHAN JOST.

**CERTIFICATE OF CORRECTION.**

Patent No. 1,823,606.

Granted September 15, 1931, to

STEPHAN JOST.

It is hereby certified that the name of the assignee in the above numbered patent was erroneously written and printed as to the firm "Farberei- & Oppretur Gesellschaft (Vormals A. Blavel & Fritz Lindenmeyer), of Basel, Switzerland", whereas said name should have been written and printed as to the firm Färberei- & Appretur Gesellschaft (Vormals A. Clavel & Fritz Lindenmeyer), of Basel, Switzerland, as shown by the records of assignments in this office; and that the said Letters Patent should be read with this correction therein that the same may conform to the record of the case in the Patent Office.

Signed and sealed this 17th day of November, A. D. 1931.

**CERTIFICATE OF CORRECTION.**

**Patent No. 1,823,606.**

**Granted September 15, 1931, to**

**STEPHAN JOST.**

**It is hereby certified that the name of the assignee in the above numbered patent was erroneously written and printed as to the firm "Farberei- & Oppretur Gesellschaft (Vormals A. Blavel & Fritz Lindenmeyer), of Basel, Switzerland", whereas said name should have been written and printed as to the firm Färberei- & Appretur Gesellschaft (Vormals A. Clavel & Fritz Lindenmeyer), of Basel, Switzerland, as shown by the records of assignments in this office; and that the said Letters Patent should be read with this correction therein that the same may conform to the record of the case in the Patent Office.**

**Signed and sealed this 17th day of November, A. D. 1931.**